

# UNITED STATES PATENT OFFICE.

FEDERICO GIOLITTI, OF TURIN, ITALY, ASSIGNOR TO SOCIETA ANONIMA ITALIANA  
GIO. ANSALDO ARMSTRONG & CO., OF GENOA, ITALY.

## PROCESS FOR THE CEMENTATION OF ARTICLES OF IRON, STEEL, AND ALLOYS OF STEEL.

1,093,844.

Specification of Letters Patent.

Patented Apr. 21, 1914.

No Drawing.

Application filed June 13, 1910. Serial No. 566,576.

To all whom it may concern:

Be it known that I, Dr. FEDERICO GIOLITTI, a subject of the King of Italy, residing at No. 105 Corso Vittorio Emanuele, 5 Turin, in the Kingdom of Italy, have invented new and useful improvements in Processes for the Cementation of Articles of Iron, Steel, and Alloys of Steel, of which the following is a specification.

10 This invention has for its object to provide an improved process for the cementation of articles of iron, steel and alloys of steel, whereby a layer of desired depth more highly carburized than the remainder of the 15 article, may be produced in the zone situated immediately below the external surface of the article.

15 The improved process consists substantially in employing "gaseous carbonic anhydrid" (hereinafter referred to as "carbon dioxide") in addition to carbon which is used in many existing cementation processes. Carbon dioxide can be obtained in commerce in great purity and at a low price.

20 The employment of carbon dioxide in the presence of wood charcoal or any other kind of carbon, allows of dispensing entirely with the use of the numerous foreign substances such as barium carbonate, alkaline cyanids, 25 ferrocyanids, nitrogenous organic substances, hydrocarbids, etc., which it has been necessary to add to wood charcoal in the usual cementation processes in order to prevent the cementation from being practically useless by reason of its extreme slowness.

The improved process may be carried out generally as follows: The articles to be cemented are placed in a fixed or movable receptacle (hereinafter referred to as the "cementing chamber") of steel plate or of refractory material of form and dimensions varying with the nature and dimensions of the said articles. In many cases small articles may be cemented in the ordinary retorts used in gas works for distilling coal in the manufacture of illuminating gas. The cementing chamber is placed in a furnace capable of heating it to a constant and uniform temperature between the limits of 50 900 and 1100 degrees centigrade. The cementing chamber is provided with a door capable of closing air-tight to allow of placing the articles to be cemented therein, and

with pipes arranged to cause a current of 55 carbon dioxide to circulate slowly through the chamber. The process is started by placing a layer of carbon in the cementing chamber. It is preferred for this purpose to use wood charcoal that has been thoroughly calcined and reduced to small pieces; this charcoal is hereinafter referred to as "granulated charcoal." The size of the pieces of the granulated charcoal and the thickness of the layer of such charcoal vary according to the varying dimensions, quantity and shape of the articles to be cemented. For instance for cementing at one operation 100 kilograms of pieces of steel not too complicated in shape, (such as for instance, ball 60 bearing races, axles of bicycle wheels, etc.,) no one piece exceeding 400 to 500 grams in weight, the charcoal must be crushed, and only that portion of it is to be used which will pass through a sieve having 26 meshes 65 to the square centimeter, but which will be retained by a sieve having 81 meshes to the square centimeter. With the said portion of the charcoal a first layer is formed having a depth of about 10 to 15 centimeters. For 70 cementing very large articles; such as for instance armor plates for ships, the charcoal must be employed in pieces of somewhat larger size and the thickness of the first layer must be increased to, for instance 75 from 40 to 50 centimeters. The articles to be cemented are then placed upon the first layer of charcoal, at a distance of from one to two centimeters apart. Any pieces which by reason of their shape or weight, have a 80 tendency to sink into the charcoal, may be easily supported in position by means of a metal netting placed underneath them. Pieces of flat or elongated form may be placed vertical. Upon the articles placed 85 as described, a quantity of granulated charcoal is poured so as to cover them completely. Upon this new layer of charcoal, other articles to be cemented are placed and covered with more granulated carbon, and 90 so on, until the cementing chamber is filled. In many cases it may be convenient for the purpose of obtaining perfect homogeneity of the cemented zone, to fix the articles to be cemented on a rotary shaft of metal or 95 refractory material which extends through the wall of the cementing chamber and can be rotated slowly.

The pure granulated charcoal prepared as described above, and duly calcined, forms (especially when it has been employed several times in the improved cementation process) a very slippery and movable mass which penetrates with the greatest ease into every recess of the articles to be cemented. This penetration may be promoted by giving slight shakes or shocks to the cementing 10 chamber.

It will be advisable to employ small granulated charcoal for cementing articles of complicated shape having small recesses, although it has been found that the gas is the 15 essential carburizing medium in the improved cementation process, and that cementation takes place equally in those parts of the steel articles which are not in contact with the charcoal, but are distant some 20 centimeters from it.

The cementing chamber having been filled in the manner described above, the charging door is closed, and a current of carbon dioxide is caused to circulate slowly 25 through the chamber by means of the pipes already referred to. The speed of the current of carbon dioxide varies also according to the depth of cementation which it is desired to produce. While the current of carbon dioxide gas is kept uniform, the temperature of the cementing chamber is raised to bright red heat and is then maintained 30 constant during the entire duration of the cementation which depends—according to fixed definite conditions that are readily determined by preliminary experiments—on the temperature, the speed of the current of gas, and the desired depth of the zone of cementation. It is impossible to give here 35 particulars suitable for all possible cases, only two of which are given here by way of example in order to show how the results of the improved process depend on the conditions under which it is performed:—

40 First example: For cementing according to the improved process at a temperature of 1000 degrees centigrade, articles composed of soft steel (containing 0.07 per cent. of carbon) in order to produce a zone of cementation having a total depth of 2.5 millimeters, the current of carbon dioxide must be caused to pass through the chamber for two hours at a speed of about 1 liter per hour 45 for each square decimeter of the external surface of the steel articles to be cemented.

Second example: By operating at a temperature of 960 degrees C., but otherwise under the conditions stated in the first example, a zone of cementation is produced 50 having a depth of 1.4 mm. The gases issuing from the cementing chamber are collected in a suitable gas holder whence they can be caused to circulate anew through the cementing chamber with an effect similar to that of the fresh carbon dioxide. This may

be repeated indefinitely, so that a great saving is effected. When the cementation is complete, the current of gas is stopped, and a trap door in the bottom of the cementing chamber is opened to allow the granulated charcoal to pass out which it does automatically and with the greatest ease owing to its extremely slippery nature; it is received in a suitable receptacle whence it can be poured directly into another cementing chamber. By this means the same charcoal may serve for a very large number of operations, since only the small amount of charcoal which serves directly to carburize the steel of the zones of cementation, is consumed. After the granular charcoal has been thus removed, the cemented articles remaining in the cementing chamber can be removed readily therefrom for the purpose of being hardened or tempered or subjected to other suitable treatment. When the chamber is empty, the next charge is made directly in the manner described above.

In many cases, and especially when it is desired to produce zones of cementation of great depth without increasing the percentage of carbon therein to a too high degree, it is advisable instead of removing the whole of the granulated charcoal from the cementing chamber in the manner hereinbefore described to remove only the quantity which is necessary to uncover the surface of the articles to be cemented, and then to continue the heating and the circulation of the current of gas in the presence of the charcoal remaining in the cementing chamber. By this means an extraordinarily uniform distribution of carbon in the zone of cementation is obtained, and the carburization may be carried to very great depths (6 or 7 centimeters) without the percentage of carbon in the zone of cementation exceeding the amount produced by the first part of the process. The same result may be produced by leaving the charcoal in the cementing chamber, and mixing a certain quantity of air with the carbon dioxide during a part or the whole of the cementation. The percentage of carbon in the zones thus produced is lower, all the other conditions being equal, the greater the proportion of air that is added to the carbon dioxide. Thus for instance in the first example, (cementation during two hours at 1000 degrees C.) by employing pure carbon dioxide a maximum percentage of 0.9 per cent. is produced in the zone of cementation, whereas by employing carbon dioxide mixed with 60 per cent. of air, the maximum percentage of carbon in the zone of cementation is reduced to 0.65 per cent.

In cases where it is desired to produce zones of cementation having a very high percentage of carbon (for instance up to 1.3

or 1.5 per cent.), it is sufficient to introduce by means of one or more pipes into the cementing chamber during the process (which is performed otherwise in the manner described above) larger or smaller quantities (according as it is desired to obtain a greater or lesser percentage of carbon) of gaseous hydrocarbons such as acetylene, ethylene, gas obtained by the distillation of coal, etc., or liquid hydrocarbons such as benzol, petroleum, etc. The gaseous hydrocarbons, or the vapors which are formed immediately by the liquid hydrocarbons at the temperature of the cementing chamber, mingle with the gases circulating in the apparatus, and have the effect of increasing the percentage of carbon in the zones of cementation. In this case it is no longer necessary that the articles to be cemented shall be in contact with the granulated charcoal. In many cases, in order to produce certain effects, it may be advisable to add air as well as hydrocarbons to the gases employed for cementation. These additions may be made either simultaneously or in succession.

The chief advantages of the improved cementation process over existing processes, either as regards its greater facility of execution, or as regards the better results produced by it, are the following:—

1. The dispensing with the existing inconvenient and expensive cementation boxes, and the use in their place, of a refractory receptacle of the retort type which can be charged and discharged by successive operations without having to be removed from the furnace.

2. Great saving of cementing material, because the same carbon dioxid gas can be employed over again indefinitely for a long succession of cementing operations, since only the small quantity of gas is consumed which is lost through leakage, and the whole of the charcoal is utilized in the carburization of the iron or steel. In other words, the cementing material does not lose its efficiency, (that is, it never becomes impoverished as is the case with the usual cementing powders), so that it can be used up completely, and not even the slightest quantity need be thrown away.

3. The speed of penetration of the carbon is far greater than that which can be obtained with all other existing processes. The extraordinary importance of this fact is evident.

4. The extraordinary uniformity of distribution of the carbon in the zones of cementation, which has a very beneficial influence upon the strength of the cemented articles.

5. The possibility of regulating the percentage of carbon in the zones of cementation in such a manner as to keep the maximum percentage below the usual limits

(which vary according to the composition of the steel to be cemented) above which a loss of strength begins to appear, and in all cases the absolute certainty of being able to avoid, if so desired, the presence of "cementite" in the zones of cementation. 70

6. The possibility of predetermining with certainty the conditions such as temperature, speed of the current of gas, etc., suitable for producing desired results, such as 75 depth of cementation, percentage of carbon, etc.

7. The possibility of producing zones of cementation of very great depths, up to beyond 6 centimeters, without having ever to 80 renew the cementing material, because, as stated above, it never becomes impoverished.

8. The absolute certainty of not introducing into the steel any foreign substance other than carbon, which is not the case with existing cementing powders containing cyanides, organic substances, etc. 85

9. The complete preservation of the surfaces of the cemented articles, which remain perfectly clean after the cementing process 90 as before it, thereby simplifying greatly rectifying operations.

10. Very slight variation in the volume of the cemented articles, thereby simplifying also considerably the work of rectifying the 95 finished articles, and sometimes rendering that work unnecessary.

Having now described my invention, what I claim as new and desire to secure by Letters Patent is:—

1. The improved process of cementing an article of iron, steel or alloy of steel, wherein the article to be cemented is heated to a temperature of from about 900 degrees to about 1100 degs. centigrade in the presence of pure 105 carbon in a state of comparatively fine subdivision and carbon dioxid, whereby said article is provided with a surface layer of any desired depth carburized to any degree more than the remainder of the article, as set 110 forth.

2. The improved process of cementing an article of iron, steel or alloy of steel, wherein the article to be cemented is packed in pure carbon in a state of comparatively fine subdivision, a current of carbon dioxid passed therethrough while heating said packed article to a temperature of from about 900 to 1100 degrees centigrade, then after a certain interval, that portion of the pure carbon which 115 is in contact with the surfaces of the article to be cemented is removed, and then the circulation of the carbon dioxid and the heating continued as before, whereby very deep zones of cementation are produced without 120 increasing unduly the percentage of carbon therein, as set forth.

3. The improved process of cementing an article of iron, steel or alloy of steel, wherein the article to be cemented is packed in gran- 130

4  
 1. The improved process of cementing an  
 5. ulated charcoal, a current of carbon dioxid  
 passed therethrough while heating said so  
 packed article to a temperature of from  
 about 900 degrees to 1100 degrees centigrade,  
 then after a certain interval, that portion of  
 the granulated charcoal which is in contact  
 with the surfaces of the article to be ce-  
 mented is removed, and then the circulation  
 of the carbon dioxid and the heating con-  
 tinued as before, whereby very deep zones of  
 10 cementation are produced without increas-  
 ing unduly the percentage of carbon therein,  
 as set forth.

4. The improved process of cementing an  
 15 article of iron, steel or alloy of steel, wherein  
 the article to be cemented is packed in pure  
 carbon in a state of comparatively fine sub-  
 division and a current of carbon dioxid  
 passed therethrough with the addition of a  
 20 certain quantity of air while heating said so  
 packed article to a temperature of from  
 about 900 degrees to 1100 degrees centigrade  
 as set forth.

5. The improved process of cementing an  
 25 article of iron, steel or alloy of steel, wherein

the article to be cemented is packed in gran-  
 ulated charcoal and a current of carbon di-  
 oxid passed therethrough with the addition  
 of a certain quantity of air while heating  
 said so packed article to a temperature of 30  
 from about 900 degrees to 1100 degrees centi-  
 grade, as set forth.

6. The improved process of cementing an  
 article of iron, steel or alloy of steel, wherein  
 the article to be cemented is packed in pure 35  
 carbon in a state of comparatively fine sub-  
 division and a current of carbon dioxid  
 passed therethrough with the addition of  
 certain quantities of vaporizable hydrocar-  
 bon and air, while heating said so packed 40  
 article to a temperature of from about 900  
 degrees to 1100 degrees centigrade, as set  
 forth.

In testimony whereof I have hereunto set  
 my hand in presence of two subscribing wit- 45  
 nesses.

DR. FEDERICO GIOLITTI.

Witnesses:

PIERO GIAUOLIO,  
 FEDERICO CARUEVATI.